

May 6, 1924.

1,492,580

A. F. SCHRAMM, JR

FABRIC BEARING DESIGN IN RELIEF

Filed Aug. 16, 1922

Fig. 1.



Fig. II



Fig. 3.



Fig. 4.



Inventor  
August F. Schramm, Jr.  
By his Attorneys  
Prindle, Wright, & Small

## UNITED STATES PATENT OFFICE.

AUGUST F. SCHRAMM, JR., OF RICHMOND HILL, NEW YORK.

## FABRIC BEARING DESIGN IN RELIEF.

Application filed August 16, 1922. Serial No. 582,329.

*To all whom it may concern:*

Be it known that I, AUGUST F. SCHRAMM, Jr., a citizen of the United States, a resident of Richmond Hill, L. I., in the county of Queens and State of New York, have invented certain new and useful Fabric Bearing Designs in Relief, of which the following is a specification.

This invention relates to a fabric bearing design in relief and an improved method for making such fabric.

The invention in its preferred form is shown in the accompanying drawings in which—

Figure 1 illustrates a piece of muslin, the upper left hand corner of which has been provided with a nap;

Fig. 2 represents a section of the muslin with the nap over the entire surface of one side;

Fig. 3 represents the muslin of Fig. 2 after it has been rolled between pressure rollers bearing a suitable design which is imparted to the muslin, and

Fig. 4 is an enlarged section on line 4—4 of Fig. 3 showing the approximate relations between the fabric, the outstanding nap, and the depressed or compressed portions of the nap.

In said drawings the muslin is represented by the numeral 1 and the nap by the numeral 2. The nap is made on the fabric by the use of a suitable picking machine which picks up from the surface of the muslin the short fibers to provide a nap on the main body of the fabric, this operation being well known in the art. After the nap is thus provided, the other side of the fabric is impregnated with a gum which is non-hygroscopic and which is plastic when heated. The gum solution is allowed to penetrate until it reaches the nap so that when the muslin fabric is compressed between the rollers the depressed or compressed portions of the nap will be glued down to the base of the fabric and will not therefore be able to resume their former position. The rollers employed are preferably internally heated so that the gum will become plastic and flow sufficiently to efficiently glue down the depressed portions of the nap. It is not desirable to allow the gum to penetrate any further so that it would be absorbed by the portions of the nap not depressed by the rollers. The latter may be

of any construction such as embossed rollers or rollers provided with designs in relief or etched designs.

As a result of this operation there is imparted to the muslin fabric a design such as shown in Fig. 3 in which numeral 3 designates the original nap or pile and numeral 4 designates the compressed or depressed portions of the original nap which are now firmly held down against the body of the fabric by the glue and by the effects of the pressure. In Fig. 4 which is an enlarged section of Fig. 3, numerals 3 at the left show the original nap which has been given a corduroy-like effect by compressing the portions designated by the numerals 5 along narrow lines as shown in Fig. 3. The circular embossments 6 appearing in Figures 3 and 4 have depressed areas 7 of the nap lying between them. The portions designated by numerals 7 in Fig. 4 are the same as portions 4 in Fig. 3. The depressed portions of the nap will not resume their original positions again under adverse conditions such as humid weather or dampness of the fabric because they are glued down by a non-hygroscopic glue. They are therefore permanently fixed to the fabric as the result of the compression.

While in the above embodiment the treatment of a muslin fabric has been described, it is to be understood that the same method may be applied to many other fabrics and fabric-like materials capable of receiving embossing by creating depressions and elevations. Thus velours, velvets and velvet-like materials having a pile as for example pile velvet or corduroy may be treated in a similar manner to provide a permanent design in relief. Fabrics and similar materials which have a natural nap or a natural pile may be thus treated without the preliminary operation of picking out a nap from the material. Cotton goods, linen, wool, and in fact various animal and vegetable fabric material may be subjected to the above described process. The process may be varied by first providing an artificial nap or pile on the paper or similar material and then glueing and running through the rollers. Besides these modifications others will suggest themselves in which it is desired to provide designs in relief by creating depressions in any suitable manner and securely fixing these depres-

sions to the base portion of the material by a suitable glue equivalent to the one above described.

In this manner there is produced an article of manufacture which will bear various designs in relief without liability of deterioration due to the tendency of the depressed portions to rise again when dampened or released from their depressed positions. Articles which are not thus treated with the gum will have a strong tendency to blur the design after a lapse of time or during humid weather because of the raising up of the depressed portions of the nap and these depressed portions would of course not resume their depressed positions again and would therefore completely ruin the effect of the design. My invention therefore provides a very superior article of manufacture which may be used for dress goods, wall paper, ornamental draperies, linings, and many other purposes.

The gum or glue above referred to may advantageously consist of the following composition: A thin solution of unvulcanized rubber in gasoline or mineral naphtha, about 20%, rosin about 5%, and gasoline or mineral naphtha about 75%. These proportions may vary, for example, the rosin may be as low as about 1% or as high as 10% but such high amounts are likely to render the goods too stiff; the rubber solution may also vary considerably, e. g., it may amount to 33%. The solvents may be replaced by others, e. g., chloroform, carbon tetrachloride, benzol, carbon disulfid, ether, oil of turpentine, and other rubber solvents. It is desired to limit the proportions so as not to make the fabric stiff, harsh, or rough; it should preferably have a soft feel and the amount of gum should accordingly be kept as low as possible.

The above gums are waterproof and non-hygroscopic and will therefore permanently hold the depressed nap down. However, in certain cases, water-soluble gums may be used such as Calcutta elastic gum which is classed as a cold water gum. This will hold the nap down fairly well. Other gums or glues may be used according to the class of goods being treated. It is preferable that the gum be non-hygroscopic, non-odorous, and colorless, and that it will not impart harshness or stiffness to the fabrics.

As many apparently widely different embodiments of this invention may be made without departing from the spirit thereof, it is to be understood that I do not intend to limit myself to the specific embodiment thereof except as indicated in the appended claims.

I claim:

1. A cloth fabric having a pile and bearing designs in relief, the depressed portions

thereof being permanently fixed to the fabric base.

2. A cloth fabric having a pile and bearing designs in relief, the depressed portions thereof being glued to the fabric with a non-hygroscopic adhesive material. 70

3. A cloth fabric having a pile and bearing designs in relief, the depressed portions of the design being permanently fixed to the fabric base by means of a non-hygroscopic adhesive material which has the 75 property of becoming plastic when heated.

4. A cloth fabric having a pile and bearing designs in relief, the depressed portions of the design being permanently fixed to the fabric base by means of an elastic 80 gum.

5. The improvement in the method of manufacturing cloth fabrics having a pile and bearing designs in relief comprising fixing depressed portions of the design to 85 the fabric by means of an adhesive material.

6. The improvement in the method of manufacturing cloth fabrics having a pile and bearing designs in relief comprising 90 fixing depressed portions of the design to the fabric by means of a non-hygroscopic adhesive material.

7. The improvement in the method of manufacturing cloth fabrics having a pile and bearing designs in relief comprising 95 fixing depressed portions of the designs to the fabric by means of a water-proof gum which is non-hygroscopic.

8. The improvement in the method of 100 manufacturing cloth fabrics having a pile and bearing designs in relief comprising fixing depressed portions of the design to the fabric by means of an elastic gum.

9. The improvement in the method of 105 manufacturing fabrics bearing designs in relief in which a fabric provided with a nap is rolled between compression rollers carrying suitable designs, characterized by applying a non-hygroscopic adhesive material to the reverse side of the fabric before the rolling operation. 110

10. The improvement in the method of manufacturing fabrics bearing designs in relief in which a fabric provided with a 115 nap is rolled between compression rollers carrying suitable designs, characterized by applying a non-hygroscopic adhesive material to the reverse side of the fabric prior to the rolling operation, said adhesive being plastic when heated, and said rollers being sufficiently heated to render the adhesive plastic.

In testimony that I claim the foregoing, I have hereunto set my hand this 15 day 125 of August, 1922.

AUGUST F. SCHRAMM, JR.